

# UNITED STATES PATENT OFFICE.

WILLIAM RICKMERS, OF LONDON, ENGLAND.

## EXPLOSIVE.

1,032,242.

Specification of Letters Patent.

Patented July 9, 1912.

No Drawing.

Application filed June 28, 1909. Serial No. 504,784.

To all whom it may concern:

Be it known that I, WILLIAM RICKMERS, a subject of the Emperor of Germany, residing at London, in England, have invented certain new and useful Improvements in Explosives, of which the following is a specification.

According to this invention the explosive compound comprises the combination of perchlorate of ammonia, a nitrate of an alkali metal either nitrate of soda or nitrate of potassium, a solid or liquid product of natural petroleum substantially non-volatile at ordinary temperatures, and a nitrated 10 coal tar product. It is convenient to proportionate the perchlorate of ammonia and the nitrate in a manner already known so that they are relatively always in the same 15 molecular proportions. Further the relative 20 quantities of carbon and oxygen in the composition must be such that as far as possible complete combustion takes place.

The following may be given as an example of the improved explosive:

|    |                        |     |
|----|------------------------|-----|
| 25 | Paraffin wax           | 13% |
|    | Trinitrotoluene        | 14% |
|    | Perchlorate of ammonia | 42% |
|    | Sodium nitrate         | 31% |

30 As indicated other hydrocarbons of a similar nature as above defined may be used alternatively the percentages varying as found desirable. In some cases one hydrocarbon may be in liquid form and combined 35 with another hydrocarbon in solid form. The explosive compound may be treated with a suitable binding medium where needed in order to enable it to be made up in a convenient state for handling. As an 40 example agar agar may be employed as a

binding medium in the proportion of .15% to .5%. The explosive may be employed in the form of powder or may be in solid form or compressed or otherwise.

What I claim as my invention and desire to secure by Letters Patent is:—

1. In a composition of matter for use as a blasting explosive, the combination of perchlorate of ammonia, a nitrate of an alkali metal, both these substances being in equal molecular proportions, a hydrocarbon of the paraffin series and a nitro-compound of the aromatic series as set forth.

2. In a composition of matter for use as a blasting explosive, the combination of perchlorate of ammonia, sodium nitrate, these two substances being in equal molecular proportions, paraffin and trinitrotoluene as set forth.

3. In a composition of matter for use as a blasting explosive, the combination of perchlorate of ammonia, sodium nitrate, these two substances being in equal molecular proportions, paraffin, trinitrotoluene and a binding medium as set forth.

4. A composition of matter for use as a blasting explosive, combined in approximately the following proportions, to wit:— 42 per cent. perchlorate of ammonia, 31 per cent. sodium nitrate, 13 per cent. paraffin 70 wax and 14 per cent. trinitrotoluene as set forth.

In testimony whereof I have signed my name to this specification in the presence of two subscribing witnesses.

WILLIAM RICKMERS.

Witnesses:

MAURICE STRODE,  
FRANK GODWIN.